

Dec. 6, 1938.

H. STRÄB ET AL

2,138,892

PROCESS FOR THE MANUFACTURE OF ELECTROSTATIC CONDENSERS

Filed April 12, 1937

Fig.1



Fig.2



Inventors  
Hermann Sträb  
Karl Reger  
Walter Dorn  
by Roy F. Stevards  
their attorney

## UNITED STATES PATENT OFFICE

2,138,892

PROCESS FOR THE MANUFACTURE OF  
ELECTROSTATIC CONDENSERS

Hermann Sträß, Stuttgart, Karl Reger, Stuttgart-Sillenbuch, and Walter Dorn, Stuttgart, Germany, assignors to Robert Bosch Gesellschaft mit beschränkter Haftung, Stuttgart, Germany

Application April 12, 1937, Serial No. 136,420  
In Germany April 16, 1936

16 Claims. (Cl. 175—41)

The present invention relates to electrostatic condensers.

The dielectrics as for example paper or the like used for the manufacture of condensers, in particular of wound condensers suffer the disadvantage that they do not have at every place of the total dielectric surface, the same resistance to break-down, but that minute holes or porous places occur, which very easily lead to the occurrence of break-down.

It is known that these bad places of the dielectric can be made less troublesome if very thin metal coatings are used, and, with the help of over voltages an artificial break-down is obtained with so great a current that this burns out the metal coating round a break-down spot. Hereby the metal coating is burnt out in a region which is larger than the hole in the dielectric.

With this process on correct choice of the metal coating, the insulation of the dielectric can be considerably improved. However there is a danger that by the break-down process, small conducting particles of carbon may be produced in the insulating material, which may produce as a consequence a certain even if small conductivity at the breakdown spots.

According to the invention this danger is overcome by not covering the dielectric with metal from the start at its weak or holed places and in their immediate vicinity. If e. g. a metal foil is used as metal coating of the condenser, those places may be cut or stamped out of the foil which come to lie on the weak places of the dielectric on building up the condenser.

For ascertaining the positions of the weak places of the dielectric air can be blown from one side against the dielectric. From the amount of the air escaping through the dielectric, the positions of the weak places may be determined. The back side of the dielectric may also be painted with a coloured or fatty coating which penetrates at the weak places, and in this manner the position of the weak places of the dielectric shows on the front side.

The weak places of the dielectric can in the simplest manner be made into places not provided with a metallic coating, if the coating of the condenser is obtained as a metal deposit directly on the dielectric for example by spraying, sputtering or evaporation. If on deposition of the metals the weak places of the dielectric and their immediate vicinity are covered by stencils preferably circular in form, then the weak places remain free of metal.

In the obtainment of a metal deposit on a pro-

gressing band of dielectric, as for example comes into question for the manufacture of wound condensers, the use of stencils is unsuitable, since the stencils must travel with the band. In this case it is preferable to apply to the weak places of the dielectric and their immediate vicinity a covering or deposition stopping material. After the metallization the covering material with the metal layer deposited thereon can be again removed. There can be used for this object also a covering material e. g. fat or the like, on which the metal deposit obtained e. g. by spraying, adheres badly. After the precipitation the badly adhering metal layer on the places covered may be wiped away.

In many cases the same result can be obtained even more simply by applying to the weak places of the dielectric or their immediate vicinity before the deposition a substance which does not at all allow the production of a metal deposit. These properties are possessed by substances which evolve vapour on heating in vacuo. If such a substance is applied to the weak places of the dielectric and the metal deposit obtained in vacuo by cathode sputtering or purely thermal metal evaporation then no metal is deposited at these places since the vapours produced there act as a protective cushion. Precipitation preventing substances of this kind are for example aliphatic or aromatic hydrocarbons and hydrocarbon-like substances such as for example, fats, oils, halogen derivatives of these hydrocarbons, alcohols (e. g. glycerin) resins, waxes, paraffins and other organic substances.

In order to obtain sharp definition of the metallized and blank spaces, it is preferable to keep the layers of covering or deposition preventing substances as thin as possible. In this manner the edges of the coating are prevented from running. This danger of the edges running is particularly great if any time elapses between the application of the covering or deposition preventing substances and the production of the metal coating. For this reason it is preferable to apply the coating or deposition preventing substances, directly before the metallization, and also in the same vessel, in which the metallization occurs.

There is another reason for applying the coating substances very thinly. Long bands of dielectric e. g. whole rolls of paper have mainly to be metallized. If it is wished to apply to the weak places of the dielectric coating or deposition preventing substances, and to roll up the long dielectric band again before the metalliza-

tion, then there exists the danger that the coating materials will leave behind traces of themselves on the neighbouring windings of the roll, and places free of metal will be caused in the 5 subsequent metallizing where these are not desired. Therefore those cases in which oil or fats are used as deposition preventing layers e. g. in metal evaporation in vacuo they must only be applied very thinly.

10 In order completely to prevent this effect on the neighbouring winding of a roll the coating or deposition preventing substances are not only applied very thinly, but also a substance is used which is solid or at least semi-solid at normal 15 temperatures.

18 In order not to affect the neighbouring windings, an additional paper strip which prevents direct contact between the front and back sides of the single windings can also be wound with 20 the treated bands.

25 The application of the coating or deposition preventing substance to the weak places of the dielectric can be very much simplified by not first investigating where the weak spots in the dielectric are, but by applying coating material in a liquid or semiliquid condition directly to the rear side of the dielectric in a similar way to what was described above for the detection of the weak spots, in such a way that they pass through the 30 weak places in the dielectric and spread out over a small range (about 1 to 5 mm. in diameter) around the weak spots. If necessary the substance applied on the back side must be kept liquid until it has penetrated to the necessary degree 35 through the dielectric by the use of high temperatures.

40 If for example fat has been applied to the back side of a paper band till it passes through the paper at the porous places, and spreads out for a certain distance on the front side of the paper band, and if the front side of this penetrated paper band is subjected in a vacuum vessel to a metal vapour then the weak places of the paper, protected by the fat, remain metal free. If the 45 fat applying and evaporating places are arranged the one immediately behind the other and the nature of the deposition preventing material, and the temperatures between application of fat and evaporating places are chosen so that this substance spreads as easily and rapidly as possible then the whole process may be carried out in a 50 single operation.

55 In Figs. 1 and 2, is shown an example of construction of a metallized condenser paper prepared in the manner described.

Figure 1 shows a view on the metallized side of the paper.

Figure 2 shows a section along the line 2—2 of Fig. 1 with a highly exaggerated view of the thicknesses.

60 In the figures *a* denotes a paper band, on which is applied a metal layer *b*, *c* are weak places in the paper. On the metallized side of the paper the metal coating is absent for a small region *d* around the weak places *c*, *f* is a metal free edge of the paper. If a second paper band is used in which the metal free edge is on the other side, then these two bands may be wound up together to a wound condenser. Whilst in normal wound 70 condensers several paper layers must always be used mutually to cover the weak places of the paper, the additional nonmetallized paper layers are in most cases not necessary in the condensers prepared according to the invention.

If the metal coating *b* is made thinner than 2 $\mu$

thus for example equal to 1 $\mu$  or 0.1 $\mu$  or less, there is obtained the advantage that the weak places of the dielectric produced somewhat with time, in the normal operation of the condenser can cause no injury. If such a condenser breaks down at a 5 weak spot, then its own energy suffices to send a short circuiting current through the break-down spot so that the metal coating vanishes on account of the local heating here produced, over a range which is larger than the break-down hole 10 in the dielectric. After such a break-down the condenser is again fully operative, and has insulated itself again automatically.

We declare, that what we claim is:

1. In a process for the manufacture of electro- 15 static condensers, the steps which comprise depositing a metal coating on a dielectric and protecting the weak places of the dielectric against the deposition of metal.

2. In a process for the manufacture of electro- 20 static condensers, the steps which comprise applying to the weak spots of a dielectric a substance which can be removed and which prevents the deposition of metal thereon, and depositing a metal coating on the dielectric. 25

3. In a process for the manufacture of electro- 30 static condensers, the steps which comprise applying to the weak spots of a dielectric a substance to which the subsequent metal coating adheres badly, depositing a metal coating on the dielectric, and removing the badly adhering portions of the coating.

4. In a process for the manufacture of electro- 35 static condensers, the steps which comprise applying to the weak spots of a dielectric and their immediate vicinity a substance capable of preventing the deposition of metal, and depositing metal on the dielectric.

5. In a process for the manufacture of electro- 40 static condensers, the steps which comprise applying to the weak spots of a dielectric and their immediate vicinity, a substance giving off vapours in vacuo, and depositing metal on the dielectric in vacuo.

6. In a process for the manufacture of electro- 45 static condensers, the steps which comprise applying a hydrocarbon like substance to the weak spots of a dielectric and their immediate vicinity, and depositing metal on the dielectric in vacuo.

7. In a process for the manufacture of electro- 50 static condensers, the steps which comprise applying a fat or oil to the weak spots of a dielectric and their immediate vicinity, and depositing metal on the dielectric in vacuo.

8. In a process for the manufacture of electro- 55 static condensers, the steps which comprise applying to the weak spots of a dielectric and their immediate vicinity, a thin coating of a substance giving off vapours in vacuo, and depositing metal on the dielectric in vacuo. 60

9. In a process for the manufacture of electro- 65 static condensers, the steps which comprise applying to the weak spots of a dielectric and their immediate vicinity, a coating of a solid or semi-solid substance giving off vapours in vacuo, and depositing metal on the dielectric in vacuo.

10. In a process for the manufacture of electro- 70 static condensers, the steps which comprise applying to the back side of a dielectric a liquid or semi-liquid substance capable of penetrating the weak spots of the dielectric and spreading in their immediate vicinity on the front side of the dielectric and of preventing the deposition of metal, and depositing metal on the front side of the dielectric. 75

11. An electrostatic condenser consisting of a metal coated dielectric, the metal of which is absent from places around the weak spots of the dielectric, the edges of the metal adjacent said weak spots being smooth and unfused. 5

12. A process for the manufacture of a metalized dielectric for electrostatic condensers comprising depositing a metal coating on the greater part of a surface of a dielectric while preventing deposit of metal on defective portions of said surface. 10

13. A process for the manufacture of a metalized dielectric for electrostatic condensers comprising applying a metallization-inhibiting substance to the weak spots of a dielectric, and applying a coating of metal to the portions of the dielectric not covered by said substance. 15

14. In a process for the manufacture of elec-

trostatic condensers, the steps which comprise applying a metal coating to a dielectric and preventing by mechanical means the application of the metal coating to weak places of the dielectric. 5

15. In a process for the manufacture of electrostatic condensers, the steps which comprise applying a metal coating to a dielectric and preventing by chemical means the application of the metal coating to weak places of the dielectric. 10

16. In a process for the manufacture of electrostatic condensers, the steps which comprise applying a metal coating to a dielectric and covering defective places of the dielectric to prevent application of metal to the covered portions of the dielectric. 15

HERMANN STRÄB.

KARL REGER.

WALTER DORN.